

## UNITED STATES PATENT OFFICE

REGINALD SCOTT DEAN, OF OAK PARK, ILLINOIS, ASSIGNOR TO WESTERN ELECTRIC COMPANY, INCORPORATED, OF NEW YORK, N. Y., A CORPORATION OF NEW YORK

## OXIDATION INHIBITOR

No Drawing.

Application filed May 12, 1924. Serial No. 712,549.

This invention relates to oxidation inhibitors and to methods for producing and applying the same.

In the heat treatment of some types of articles, it is often desirable to obtain as complete protection against oxidation as possible. For example, tools having carefully ground edges or dies possessing delicately carved surfaces, are very easily ruined by oxidation 10 during heat treatment.

The method of manufacturing such dies or tools is to form them from untreated and unhardened steel and then to heat-treat them to cause a hardening of the finished article. 15 During the hardening treatment, it is desirable to avoid conditions which will make it necessary to do any work on the article after it has been hardened. For example, if the article is oxidized to any extent during the

20 hardening thereof, it is necessary to re-grind or re-touch the oxidized portions, and this may be a difficult and expensive operation. Moreover, if the article is very delicately made even a small amount of oxidation will 25 sometimes ruin it, since it may be impossible to repair the damage which has been done.

Various methods have been employed for the purpose of protecting surfaces of such articles during heat treatment. A method 30 which has been employed frequently is to sprinkle dry boric oxide on the surface to be protected. This material fuses at a comparatively low temperature and when fused is supposed to spread in the form of a film 35 over the surface in such a way as to prevent contact of the surface with the oxygen of the air.

This method is not entirely desirable because the boric oxide will usually sputter and crack off in spots when it is heated. In order to prevent this, it is necessary to use a great bulk of the protecting material so as to make a thick layer over the whole article. 40

45 Even this thick layer does not always provide uniform protection, because in some places, for instance, vertical surfaces, the protecting material does not always adhere well. In addition, boric oxide is fairly expensive, and 50 it is desirable from an economic standpoint

to use as small an amount of it as is safe and practicable.

One object of this invention is to provide an improved method for protecting material during heat treatment. 55

Another object of this invention is to provide a method for applying a uniform coating of a fusible material to the surface of an article to be heat-treated.

A further object of this invention is to 60 produce a solution consisting of a fusible material in a volatile solvent and adapted to be applied to a metallic surface for the purpose of protecting said surface during heat treatment. 65

The principal feature of this invention is forming a suspension of fusible material in a volatile solvent, applying the resulting solution to a metallic surface and allowing said solution to dry before heating the metallic 70 surface.

Other objects and features of the invention will appear more fully in the following description and will be particularly pointed out in the appended claims. 75

The first step in the process consists in providing a suspension of fusible material in a volatile carrier. The principal point to be observed in this process is to have the resulting colloidal solution practically non-aqueous, because if water is present, the liquid film will sputter and crack off of the surface to be protected while it is being heated. It is necessary to employ, therefore, a water-free solid material and a non-aqueous liquid. 80 However, to obtain a true suspension a very small amount of water is preferably present. One manner in which this water may be introduced will be explained hereinafter. As stated, the solid material employed is preferably entirely free from water, even water of crystallization. Boric oxide is a dry material and can, therefore, be used, but a fusible salt, for instance, containing water in chemical combination must be thoroughly dehydrated 85 before it is suitable for use.

The carrier liquid may be any non-aqueous, volatile, non-corrosive one and a suitable commercial liquid of this type is carbon-tetrachloride. This compound, as furnished 90

commercially, is practically free from water and will not corrode metals. Boric oxide or boric anhydride and carbon-tetrachloride may, therefore, be used together, but in combining them, the following procedure is preferably used:

First, the boric anhydride is thoroughly dried and ground very fine. It is then mixed with the carbon-tetrachloride in any desirable proportions. One part of boric anhydride and 20 parts, by weight, of carbon-tetrachloride have been found to give good results. A peptizing agent is then added to the mixture for the purpose of facilitating the formation of a colloidal solution. A small amount of aqueous alcohol, employed in the proportion of about 1% of the mixture, is found to be a good peptizing agent for use with boric oxide, or boric anhydride and carbon-tetrachloride. Chemically pure or absolute alcohol is not desirable for this purpose, however, on account of its deficiency in water. As indicated above a small amount of water is necessary to obtain a suspension of the boric oxide in the carbon-tetrachloride, and the best way of adding this water seems to be in the form of an impurity in alcohol.

A composition formed in this manner will remain in suspension for about six months if left quietly, and even if the boric oxide does settle to the bottom of the container, it can be made to re-enter into suspension by agitating the container.

This solution can be either sprayed, painted or dipped or otherwise applied to the surface which it is desired to protect. When the carbon-tetrachloride evaporates it leaves a thin film of boric oxide covering the entire surface of the article to be protected. Vertical surfaces receive the same coating as horizontal surfaces and the boric oxide applied in this manner is not dislodged or shaken off by ordinary handling. When the articles to be treated are coated in the manner just described the boric oxide film melts when heated and forms a thin fused film on the entire surface. This film will not sputter or crack; or flow in such a way as to leave vertical surfaces bare and unprotected. The most delicately formed surfaces may be sprayed with the solution and positive protection afforded to every little crevice or edge so as to render unnecessary any "touching up" after the completion of the heat treatment.

It is to be understood that the invention is not restricted to the use of a solution of boric oxide, carbon-tetrachloride and alcohol in the manner described and the invention is limited only by the scope of the appended claims.

What is claimed is:

1. An oxidation inhibitor comprising boric anhydride, carbon-tetrachloride, and a small amount of aqueous alcohol.
2. A new composition of matter comprising a stable suspension of boric anhydride,

carbon-tetrachloride and an aqueous peptizing agent.

3. A new composition of matter comprising a colloidal solution of boric anhydride, carbon-tetrachloride, and about 1% of aqueous alcohol.

4. A new composition of matter comprising a stable suspension of boric anhydride, carbon tetrachloride, and about 1% of an aqueous peptizing agent.

In witness whereof, I hereunto subscribe my name this 1st day of May, A. D. 1924.

REGINALD SCOTT DEAN.

80

85

90

95

100

105

110

115

120

125

130